# EUROPEAN PATENT SPECIFICATION

(11) **EP 1 541 711 B1**
(45) Date of publication and mention of the grant of the patent: **31.03.2010**
(21) Application number: 04257590.2
(22) Date of filing: 06.12.2004
(51) Int. Cl.: C23C 28/00

(54) **Method for preparing an article protected by a thermal barrier coating having a cerium (4+) oxide-enriched surface**
Verfahren zur Herstellung von einem Artikel geschützt mit einer Wärmedämmungsschicht, die eine mit Ceriumoxid (4+) angereicherte Oberfläche hat
Procédé pour produire un article protégé par un revêtement barrière thermique avec une surface enrichie en oxyde de cerium (4+)

(30) Priority: 12.12.2003 US 735370
(43) Date of publication of application: 15.06.2005
(73) Proprietor: GENERAL ELECTRIC COMPANY, Schenectady, NY 12345 (US)
(72) Inventor: Ackerman, John Frederick, Laramie, Wyoming 82070 (US); Darolia, Ramgopal, West Chester, Ohio 45069 (US); Boutwell, Brett Allen Rohrer, Liberty Township, Ohio 45011 (US); Venkataramani, Venkat Subramanian, Clifton Park, New York 12065 (US); Spitsberg, Irene, Loveland, Ohio 45140 (US)
(74) Representative: Szary, Anne Catherine

(56) References cited:
- EP-A- 1 295 965
- EP-A- 1 304 397
- EP-A- 1 327 704
- WO-A-02/27066
- US-B1- 6 187 453
- US-B1- 6 296 945

## Description

This invention relates to the thermal barrier coating used to protect an article such as a nickel-base superalloy substrate and, more particularly, to the inhibiting of the sintering between the grains of the thermal barrier coating.

A thermal barrier coating system may be used to protect the components of a gas turbine engine that are subjected to the highest temperatures. The thermal barrier coating system usually includes a bond coat that is deposited upon a superalloy substrate, and a ceramic thermal barrier coating that is deposited upon the bond coat. The thermal barrier coating acts as a thermal insulator against the heat of the hot combustion gas. The bond coat bonds the thermal barrier coating to the substrate and also inhibits oxidation and corrosion of the substrate.

The currently preferred thermal barrier coating is yttria-stabilized zirconia (YSZ), which is zirconia (zirconium oxide) with from about 2 to about 12 percent by weight yttria (yttrium oxide). The yttria is present to stabilize the zirconia against phase changes that otherwise occur as the thermal barrier coating is heated and cooled during fabrication and service. The YSZ is deposited by a physical vapor deposition process such as electron beam physical vapor deposition. In this deposition process, the grains of the YSZ form as columns extending generally outwardly from and perpendicular to the surfaces of the substrate and the bond coat.

When the YSZ is initially deposited, there are small gaps between the generally columnar grains. On examination at high magnification, the generally columnar grains are seen to have a somewhat feather-like morphology characterized by these gaps oriented over a range of angles relative to the substrate surface. The gaps serve to accommodate the transverse thermal expansion strains of the columnar grains and also act as an air insulator in the insulator structure. As the YSZ is exposed to elevated temperatures during service, these gaps close by a surface-diffusion sintering mechanism. As a result, the ability of the YSZ to accommodate thermal expansion strains is reduced, and the thermal conductivity of the YSZ increases by about 20 percent or more. The as-deposited thickness of the YSZ must therefore be greater than would otherwise be desired, to account for the loss of insulating capability associated with this rise in thermal conductivity during service.

It has been recognized that the addition of sintering inhibitors to the YSZ reduces the tendency of the gaps between the columnar grains to close by sintering during service of the thermal barrier coating. A number of sintering inhibitors have been proposed. However, these sintering inhibitors have various shortcomings, and there is a need for more effective sintering inhibitors. The present invention fulfills this need, and further provides related advantages.

US-B1-6296945 discloses a turbine component comprising a metal alloy substrate and a columnar thermal barrier coating on the substrate surface, the coating having (a) a columnar-grained ceramic oxide structural base material and (b) a heat resistant ceramic oxide sheath material covering the columns of the base, where the sheath comprises the reaction product of a ceramic oxide precursor sheath material which consists essentially of the composition C_{z}O_{w} and the ceramic oxide columnar structural material which consists essentially of the composition (A,B)ₓO_{y}, where A and B are selected from stable oxides which will react with C_{z}O_{w}, and C is selected from stable oxides that will react with (A,B)ₓO_{y}.

The present invention provides a method for the fabrication of an article protected by a thermal barrier coating system. The thermal barrier coating includes an effective sintering inhibitor that slows or prevents the closure of the gaps between the columnar grains. The sintering inhibitors are readily introduced into the thermal barrier coating by an infiltration technique.

The method for preparing a protected article comprises the steps of providing the article, depositing a bond coat onto an exposed surface of the article, and producing a thermal barrier coating (TBC) on an exposed surface of the bond coat. The thermal barrier coating is produced by the steps of depositing a primary ceramic coating onto an exposed surface of the bond coat, depositing a cerium-oxide-precursor compound onto the exposed surface of the primary ceramic coating, preferably so that it infiltrates into the exposed surface of the primary ceramic coating, and heating the cerium-oxide-precursor compound in an oxygen-containing atmosphere to form cerium oxide in the 4+ valence state adjacent to the exposed surface of the primary ceramic coating. As used herein, "cerium oxide" includes the simple CeO₂ (ceria) oxide, and also more-complex oxide compounds such as CeTaO₄, CeAlO₃, and CaCeO₃ (but does not include compounds of cerium with zirconium or yttrium). In each case, the cerium is in the +4 valence state. The thermal barrier coating thus comprises a primary ceramic coating on the exposed surface of the bond coat, and a sintering-inhibitor region at a surface of the primary ceramic coating. The sintering-inhibitor region comprises cerium oxide in a concentration greater than a general cerium oxide concentration in the primary ceramic coating.

The article is preferably a component of a gas turbine engine, such as a turbine blade or vane. The article is preferably made of a nickel-base superalloy.

The bond coat is preferably a diffusion aluminide or an aluminum-containing overlay bond coat.

The primary ceramic coating is preferably yttria-stabilized zirconia, typically with about 7 weight percent yttria, balance zirconia.

The cerium-oxide-precursor compound may be of any operable type that is not initially cerium oxide but is reacted to cerium oxide during processing. The preferred cerium-oxide-precursor compound is (NH₄)Ce(SO₄)₃.

The cerium-oxide-precursor compound reacts to form cerium (+4) oxide, CeO₂, rather than a more-complex compound such as a perovskite or a pyrochlore. When yttria is added to zirconia, it produces an excess of oxygen vacancies, which allows oxygen to rapidly diffuse through the thermal barrier coating. The formation of CeO₂ with cerium in the +4 valence state acts to remove the oxygen vacancies to thereby slow the diffusion of oxygen anions through the ceramic. The reduction in oxygen diffusion impedes the sintering behavior of the ceramic structure. Sintering is a surface-diffusion-related phenomenon, and the cerium oxide provides a sinter-inhibiting layer at the surface of the primary ceramic coating rather than distributed throughout the primary ceramic coating.

Other features and advantages of the present invention will be apparent from the following more detailed description of the preferred embodiment, taken in conjunction with the accompanying drawings, which illustrate, by way of example, the principles of the invention, and in which:
Figure 1 is a block flow diagram of an approach for practicing the invention;
Figure 2 is a perspective view of a turbine blade;
Figure 3 is an enlarged sectional view of the surface region of the airfoil portion of the turbine blade, taken along line 3-3; and
Figure 4 is an enlarged detail of Figure 3, taken in region 4.

Figure 1 depicts a preferred embodiment of one approach for practicing the invention. An article is provided, step 20. The article is preferably a component of a gas turbine engine, such as a turbine blade or a turbine vane. An example of such an article 40 is a gas turbine blade 42 illustrated in Figure 2. The gas turbine blade 42 has an airfoil 44 against which a flow of hot combustion gas impinges during service operation, a downwardly extending shank 46, and an attachment 48 in the form of a dovetail which attaches the gas turbine blade 42 to a gas turbine disk (not shown) of the gas turbine engine. A platform 50 extends transversely outward at a location between the airfoil 44, on the one hand, and the shank 46 and the attachment 48, on the other hand. There may be internal cooling passages through the interior of the gas turbine blade 42, ending in openings 52 on the airfoil 44 and/or at the tip 54 of the gas turbine blade 42. The gas turbine blade 42 may have a random polycrystalline grain structure, but more preferably it has a single-crystal or directionally oriented polycrystal grain structure.

The gas turbine blade 42 is preferably made of a nickel-base superalloy. As used herein, "nickel-base" means that the composition has more nickel by weight present than any other element. The nickel-base superalloys are typically of a composition that is strengthened by the precipitation of gamma-prime phase or a related phase. A typical nickel-base superalloy falls within a composition range, in weight percent, of from about 4 to about 20 percent cobalt, from about 1 to about 10 percent chromium, from about 5 to about 7 percent aluminum, from 0 to about 2 percent molybdenum, from about 3 to about 8 percent tungsten, from about 4 to about 12 percent tantalum, from 0 to about 2 percent titanium, from 0 to about 8 percent rhenium, from 0 to about 6 percent ruthenium, from 0 to about 1 percent niobium, from 0 to about 0.1 percent carbon, from 0 to about 0.01 percent boron, from 0 to about 0.1 percent yttrium, from 0 to about 1.5 percent hafnium, balance nickel and incidental impurities, although nickel-base superalloys may have compositions outside this range. A nickel-base superalloy of particular interest is Rene® N5, a registered trademark assigned to Teledyne Industries, Inc., of Los Angeles, CA, having a nominal composition in weight percent of about 7.5 percent cobalt, about 7.0 percent chromium, about 1.5 percent molybdenum, about 5 percent tungsten, about 3 percent rhenium, about 6.5 percent tantalum, about 6.2 percent aluminum, about 0.15 percent hafnium, about 0.05 percent carbon, about 0.004 percent boron, about 0.01 percent yttrium, balance nickel and minor elements.

A bond coat 60 is deposited onto an exposed surface 62 of the article 40, step 22, see Figure 3. (As used herein, an "exposed surface" is a surface which is initially exposed and not contacting anything else, and upon which a layer or coating is deposited. After the deposition, the previously exposed surface is no longer exposed, but is covered with the layer or coating.) The bond coat 60 may be of any operable type. The bond coat 60 may be a diffusion aluminide bond coat, produced by depositing an aluminum-containing layer onto the free surface 62 and interdiffusing the aluminum-containing layer with the article 40 to produce an additive layer and a diffusion zone. The bond coat 60 may be a simple diffusion aluminide, or it may be a more-complex diffusion aluminide wherein another layer, preferably platinum, is first deposited upon the surface 62, and the aluminum-containing layer is deposited over the first-deposited layer. In either case, the aluminum-containing layer may be doped with other elements that modify the bond coat 60.

The bond coat 60 may instead be an overlay coating such as an MCrAlX coating. The terminology "MCrAlX" is a shorthand term of art for a variety of families of overlay bond coats 60 that may be employed as environmental coatings or as bond coats in thermal barrier coating systems. In this and other forms, M refers to nickel, cobalt, iron, and combinations thereof. In some of these protective coatings, the chromium may be omitted. The X denotes elements such as hafnium, zirconium, yttrium, tantalum, rhenium, ruthenium, palladium, platinum, silicon, titanium, boron, carbon, and combinations thereof. Specific compositions are known in the art. Some examples of MCrAlX compositions include, for example, NiAlCrZr and NiAlZr, but this listing of examples is not to be taken as limiting. In both cases of diffusion aluminide and overlay bond coats, the bond coat 60 is typically from about 0.00127 to about 0.0254 cm (0.0005 to about 0.010 inch) thick. Such bond coats 60 and their deposition procedures are generally known in the art.

Because the platinum-aluminide diffusion aluminide is preferred, its deposition will be described in more detail. A platinum-containing layer is first deposited onto the exposed surface 62 of the article 40. The platinum-containing layer is preferably deposited by electrodeposition. For the preferred platinum deposition, the deposition is accomplished by placing a platinum-containing solution into a deposition tank and depositing platinum from the solution onto the exposed surface 62 of the article 40. An operable platinum-containing aqueous solution is Pt(NH₃)₄HPO₄ having a concentration of about 4-20 grams per liter of platinum, and the voltage/current source is operated at about 1/2-10 amperes per square foot of facing article surface. The platinum first coating layer, which is preferably from about 1 to about 6 micrometers thick and most preferably about 5 micrometers thick, is deposited in 1-4 hours at a temperature of 88-93°C (190-200°F).

A layer comprising aluminum and any modifying elements is deposited over the platinum-containing layer by any operable approach, with chemical vapor deposition preferred. In that approach, a hydrogen halide activator gas, such as hydrogen chloride, is contacted with aluminum metal or an aluminum alloy to form the corresponding aluminum halide gas. Halides of any modifying elements are formed by the same technique. The aluminum halide (or mixture of aluminum halide and halide of the modifying element, if any) contacts the platinum-containing layer that overlies the surface 62 of the article 40, which serves as the deposition substrate, depositing the aluminum thereon. The deposition occurs at elevated temperature such as from about 996 to about 1079°C (1825°F to about 1975°F) so that the deposited aluminum atoms interdiffuse into the surface 62 of the article 40 during a 4 to 20 hour cycle.

A thin aluminum oxide (alumina, Al₂O₃) scale forms on an exposed surface 66 of the bond coat 60 by oxidation of the aluminum that is in the bond coat 60 at its exposed surface 66. The aluminum oxide is a protective oxide that inhibits further oxidation of the bond coat 60. The aluminum oxide scale may be formed by reaction with residual oxygen during fabrication, or during service of the article, or both.

A thermal barrier coating 64 is produced on the exposed surface 66 (and overlying the thin aluminum oxide scale) of the bond coat 60, step 24. The production of the thermal barrier coating 64 includes first depositing a primary ceramic coating 68 onto the exposed surface 66 of the bond coat 60, step 26. The primary ceramic coating 68 is deposited, step 26, preferably by a physical vapor deposition process such as electron beam physical vapor deposition (EBPVD) or by air plasma spray (APS). The primary ceramic coating 68 is preferably from about 0.00762 to about 0.0254 cm (0.003 to about 0.010 inch) thick, most preferably about 0.0127 cm (0.005 inch) thick. The primary ceramic coating 68 is preferably yttria-stabilized zirconia (YSZ), which is zirconium oxide containing from about 2 to about 12 weight percent, more preferably from about 4 to about 8 weight percent, most preferably about 7 percent, of yttrium oxide. Other operable ceramic materials may be used as well. Examples include yttria-stabilized zirconia, which has been modified with additions of "third" oxides such as lanthanum oxide, ytterbium oxide, gadolinium oxide, neodymium oxide, tantalum oxide, or mixtures of these oxides, which are co-deposited with the YSZ.

As illustrated schematically in Figures 3 and 4 (an enlargement of a portion of Figure 3), when prepared by a physical vapor deposition process the primary ceramic coating 68 is formed primarily of a plurality of columnar grains 70 of the ceramic material that are affixed at their roots to the bond coat 60 (and to the alumina scale that forms on the bond coat 60). The columnar grains 70 of the primary ceramic coating 68 have exposed surfaces 72. As seen in Figure 4, the sides of the columnar grains 70 tend to be somewhat featherlike in morphology. There are gaps 74, whose size is exaggerated in Figures 3 and 4 for the purposes of illustration, between the facing exposed surfaces 72 of the columnar grains 70.

This morphology of the primary ceramic coating 68 is beneficial to the functioning of the thermal barrier coating 64. The gaps 74 are filled with air, which when relatively stagnant between the grains 70 is an effective thermal insulator, aiding the thermal barrier coating 64 in performing its primary role. Additionally, the gaps 74 allow the article 40, the bond coat 60 with its alumina scale, and the thermal barrier coating 64 to expand and contract in a transverse direction 76 that is locally parallel to the plane of the surface 62. Absent the gaps 74, the in-plane thermal stresses (i.e., parallel to the transverse direction 76) that are induced in the thermal barrier coating 64 as the article 40 is heated and cooled are developed across the entire extent of the thermal barrier coating 64. The thermal barrier coating 64, being a ceramic, has a generally low ductility so that the accumulated stresses would be more likely to cause premature failure. With the gaps 74 present, as illustrated, the in-plane stresses in the thermal barrier coating 64 are developed across only one or at most a group of a few of the columnar grains 70. That is, all of the grains 70 have in-plane stresses, but the magnitude of the in-plane stresses is relatively low because the strains do not accumulate over long distances. The result is that the thermal barrier coating 64 with the columnar grains 70 and gaps 74 is less likely to fail by in-plane overstressing during service.

During the exposure to elevated temperature of the article 40 during service, the facing exposed surfaces 72 tend to grow toward each other. Upon contact, the surfaces 72 sinter together by a mechanism that requires surface diffusion as one step thereof. The sizes of the gaps 74 are gradually reduced and eventually eliminated. The beneficial effects discussed above are thereby gradually reduced and eventually lost.

The present approach provides for depositing a cerium-oxide-precursor compound 78 onto the exposed surface 72 of the primary ceramic coating 68 and infiltrating the cerium-oxide-precursor compound 78 into the exposed surface 72 and thence into the near-surface regions of the primary ceramic coating 68, step 28. As used herein, "cerium oxide" includes the simple CeO₂ oxide, and also more-complex oxide compounds such as CeTaO₄, CeAlO₃, and CaCeO₃ (but does not include compounds of cerium with zirconium or yttrium). In each case, the cerium is in the +4 valence state. The cerium-oxide-precursor compound 78 is preferably (NH₄)Ce(SO₄)₃ (ammonium cerium sulfate). Examples of some other operable precursor compounds include soluble inorganic acid salts such as cerous sulfate, cerous nitrate, and cerous chloride; carboxylates of cerium such as the acetate, citrate, and tartarate; and metallo-organic complexes of cerium such as alkoxides, alkoxy carboxylates, and acetyl acetonates. The preferred cerium-oxide-precursor compound, (NH₄)Ce(SO₄)₃, is preferably provided as an aqueous solution that is contacted to the free surfaces 72 of the primary ceramic coating 68.

The cerium-oxide-precursor compound 78 is heated, step 30, in an oxygen-containing atmosphere to further infiltrate the cerium-oxide-precursor compound 78 into the primary ceramic coating 68 and to chemically react the cerium-oxide-precursor compound 78 to form cerium (valance +4) oxide, CeO₂, adjacent to the exposed surface 72 of the primary ceramic coating 68. The cerium-oxide-precursor compound reacts to form cerium (+4) oxide, CeO₂, rather than a more-complex compound such as a perovskite or a pyrochlore. When yttria is added to zirconia, it produces an excess of oxygen vacancies, which allows oxygen to rapidly diffuse through the thermal barrier coating. The formation of CeO₂ or other +4 cerium oxide acts to remove the oxygen vacancies to thereby slow the diffusion of oxygen anions through the ceramic. The reduction in oxygen diffusion impedes the sintering behavior of the ceramic structure. The CeO₂ sintering inhibitor thereby slows and preferably prevents the sintering process, which reduces and eventually eliminates the gaps 74. The oxidation step 30 is optional, because the thermal barrier coating 64 is normally subsequently heated in air during service in any event.

In a preferred approach, a 1 molar aqueous solution of (NH₄)Ce(SO₄)₃ is impregnated into the columnar structure of the thermal barrier coating 64 by dipping the article with the thermal barrier coating 64 thereon into the solution. The wet-coated part is dried at elevated temperature (e.g., 100°C) and thereafter further heated to a higher temperature (e.g., 800-1000°C) to decompose the compound to form a cerium oxide-enriched region (also denominated as element 78) overlying and contacting the primary ceramic coating 68. The cerium-oxide-enriched region serves as a sintering-inhibitor region to inhibit sintering of the primary ceramic coating 68 and thence the closing of the gaps 74. The sintering-inhibitor region comprises cerium oxide in a concentration greater than a general cerium oxide concentration in the primary ceramic coating. The thickness of the cerium oxide region may be controlled by varying the concentration of the cerium ion in the aqueous solution, and/or by performing multiple dipping and drying cycles.

In the past, it has been known to provide cerium oxide generally uniformly through a primary ceramic coating. An example is the zirconium oxide primary ceramic coating having cerium oxide mixed therein. This approach is not within the scope of the present approach, inasmuch as it does not produce a high concentration of the cerium oxide at the exposed surfaces 72 of the primary ceramic coating 68.

## Claims

1. A method for preparing a protected article (40), comprising the steps of providing the article (40);
depositing a bond coat (60) onto an exposed surface (62) of the article (40); and
producing a thermal barrier coating on an exposed surface (66) of the bond coat (60), wherein the step of producing the thermal barrier coating includes the steps of
depositing a primary ceramic coating (68) onto the exposed surface (66) of the bond coat (60),
depositing a cerium-oxide-precursor compound onto an exposed surface (72) of the primary ceramic coating (68), and
heating the cerium-oxide-precursor compound in an oxygen-containing atmosphere to form cerium oxide with the cerium in the +4 valence state adjacent to the exposed surface (72) of the primary ceramic coating (68).

2. The method of claim 1, wherein the step of providing the article (40) includes the step of
providing the article (40) as a nickel-base superalloy article (40).

3. The method of claim 1, wherein step of providing the article (40) includes the step of
providing the article (40) in the form of a component of a gas turbine engine.

4. The method of claim 1, wherein the step of depositing the bond coat (60) includes the step of
depositing a diffusion aluminide or an aluminum-containing overlay bond coat (60).

5. The method of claim 1, wherein the step of depositing the primary ceramic coating (68) includes the step of
depositing yttria-stabilized zirconia as the primary ceramic coating (68).

6. The method of claim 1, wherein the step of depositing the cerium-oxide-precursor compound includes the step of
furnishing (NH₄)Ce(SO₄)₃ as the cerium-oxide-precursor compound.

7. The method of claim 1, wherein the step of depositing the cerium-oxide-precursor compound includes the step of
infiltrating the cerium-oxide-precursor compound into the exposed surface (72) of the primary ceramic coating (68),

## Patentansprüche

1. Verfahren zum Herstellen eines geschützten Gegenstandes (40), umfassend die Stufen
Bereitstellen des Gegenstandes (40),
Abscheiden eines Bindeüberzuges (60) auf einer ausgesetzten Oberfläche (62) des Gegenstandes (40) und
Erzeugen eines Wärmesperrenüberzuges auf einer ausgesetzten Oberfläche (66) des Bindeüberzuges (60),
wobei die Stufe des Erzeugens des Wärmesperrenüberzuges die Stufen einschließt,
Abscheiden eines primären Keramiküberzuges (68) auf der ausgesetzten Oberfläche (66) des Bindeüberzuges (60),
Abscheiden einer Ceroxid-Vorstufenverbindung auf einer ausgesetzten Oberfläche (72) des primären Keramiküberzuges (68) und
Erhitzen der Ceroxid-Vorstufenverbindung in einer Sauerstoff enthaltenden Atmosphäre, um Ceroxid mit Cer im Wertigkeitszustand +4 benachbart der ausgesetzten Oberfläche (72) des primären Keramiküberzuges (68) zu bilden.

2. Verfahren nach Anspruch 1, worin die Stufe des Bereitstellens des Gegenstandes (40) die Stufe des Bereitstellens des Gegenstandes (40) als ein Superlegierungs-Gegenstand (40) auf Nickelbasis einschließt.

3. Verfahren nach Anspruch 1, worin die Stufe des Bereitstellens des Gegenstandes (40) die Stufe des Bereitstellens des Gegenstandes (40) in der Form einer Komponente eines Gasturbinen-Triebwerkes einschließt.

4. Verfahren nach Anspruch 1, worin die Stufe des Abscheidens des Bindeüberzuges (60) die Stufe des Abscheidens eines Diffusionsaluminids oder eines Aluminium enthaltenden Deck-Bindeüberzuges (60) einschließt.

5. Verfahren nach Anspruch 1, worin die Stufe des Abscheidens des primären Keramiküberzuges (68) die Stufe des Abscheidens von Yttriumoxid-stabilisiertem Zirkoniumdioxid als dem primären Keramiküberzug (68) einschließt.

6. Verfahren nach Anspruch 1, worin die Stufe des Abscheidens der Ceroxid-Vorstufenverbindung die Stufe des Lieferns von (NH₄)Ce(SO₄)₃ als Ceroxid-Vorstufenverbindung einschließt.

7. Verfahren nach Anspruch 1, worin die Stufe des Abscheidens der Ceroxid-Vorstufenverbindung die Stufe des Infiltrierens der Ceroxid-Vorstufenverbindung in die ausgesetzte Oberfläche (72) des primären Keramiküberzuges (68) einschließt.

## Revendications

1. Procédé de préparation d'un article protégé (40), comprenant les étapes de production de l'article (40) ;
dépôt d'un revêtement de liaison (60) sur une surface exposée (62) de l'article (40) ; et
production d'un revêtement formant barrière thermique sur une surface exposée (66) du revêtement de liaison (60), dans lequel l'étape de production de revêtement formant barrière thermique comporte les étapes de :
dépôt d'un revêtement céramique primaire (68) sur la surface exposée (66) du revêtement de liaison (60),
dépôt d'un composé précurseur d'oxyde de cérium sur une surface exposée (72) du revêtement céramique primaire (68), et
chauffage du composé précurseur d'oxyde de cérium dans une atmosphère contenant de l'oxygène afin de former de l'oxyde de cérium avec le cérium dans l'état de valence +4 de manière adjacente à la surface exposée (72) du revêtement céramique primaire (68).

2. Procédé selon la revendication 1, dans lequel l'étape de production de l'article (40) comporte l'étape de :
production de l'article (40) sous forme d'un article en superalliage à base de nickel (40).

3. Procédé selon la revendication 1, dans lequel l'étape de production de l'article (40) comporte l'étape de
production d'un article (40) sous la forme d'un composant d'un turbomoteur à gaz.

4. Procédé selon la revendication 1, dans lequel l'étape de dépôt de revêtement de liaison (60) comporte l'étape de
dépôt d'un revêtement de liaison à base d'aluminiure à diffusion ou de couche contenant de l'aluminium (60).

5. Procédé selon la revendication 1, dans lequel l'étape de dépôt du revêtement en céramique primaire (68) comporte l'étape de
dépôt de zircone stabilisée à l'oxyde d'yttrium pour le revêtement céramique primaire (68).

6. Procédé selon la revendication 1, dans lequel l'étape de dépôt du composé précurseur d'oxyde de cérium comporte l'étape de :
introduction de (NH₄)Ce(SO₄)₃ pour le composé précurseur d'oxyde de cérium.

7. Procédé selon la revendication 1, dans lequel l'étape de dépôt du composé précurseur d'oxyde de cérium comporte l'étape de :
infiltration du composé précurseur d'oxyde de cérium dans la surface exposée (72) du revêtement céramique primaire (68).
